

## UNITED STATES PATENT OFFICE

REED P. ROSE, OF JACKSON HEIGHTS, AND HAROLD E. CUDE, OF FLORAL PARK, NEW YORK, ASSIGNORS TO GENERAL RUBBER COMPANY, OF NEW YORK, N. Y., A CORPORATION OF NEW JERSEY

## INSULATING PAPER

No Drawing.

Application filed July 30, 1927. Serial No. 209,636.

This invention relates to improvements in the manufacture of fibrous sheet insulating materials, and particularly to the manufacture of papers for insulating purposes of various sorts.

The principal object of the invention is to produce a flexible insulating sheet material. Another object is to provide an insulating paper having high dielectric strength, flexibility, surface drag, and tensile strength. A further object is to provide a rapid method of hydrating paper pulp. Another object is to provide an insulating material which may be molded or shaped in any desired form.

The invention comprises beating a paper making fibre to a jelly-like state, combining therewith normally beaten fibre, and making into sheets. The invention includes beating paper making fibre to a jelly-like stage in the presence of chemical reagents. The invention also includes incorporating rubber from any kind of a dispersion with the beaten fibre.

As one illustration of a method of carrying out the invention, a bleached or unbleached sulphite pulp is employed. Preferably this pulp is cooked according to the Mitscherlich process in which the pulp is cooked slowly at a low temperature in the presence of sulphur dioxide and calcium carbonate. A quantity of this pulp is placed in a beater and beaten until it has assumed a jelly-like state. Ordinarily this requires from eight to ten hours, using a Mitscherlich pulp. Another quantity of kraft fibre is beaten separately in accordance with the normal procedure for making paper. A mixture of 60% by weight of normally beaten kraft and 40% by weight of the jelly-like product is then made, for instance in the beater in which the jelly-like product has been prepared, and after thorough mixing, is run through the customary paper making operations. If desired that portion of the fibre which is to receive a normal amount of beating may be added directly to the beater in which the other portion of the fibre has already been reduced at least in part to a highly gelatinized condition.

The above procedure furnishes a non-porous sheet material having an extremely close formation. The sheet or the paper possesses a high degree of strength, due to the large percentage of normally beaten fibre present in the sheet. At the same time the presence of the gelatinized fibre serves to close up the interstices in the sheet in a manner which is not possible in ordinary paper. The dielectric strength of this product is considerably greater than that of paper made in the usual way. Sheets and paper prepared by this process can be made on any standard type of paper machinery. For light weights of paper, (for example thicknesses of 0.01 inches) machines of the Fourdrinier and cylinder type may be used and in some cases the wet machine, while for the heavier weights and in cases where sheets of considerable thickness are desired, very good results may be obtained with a standard wet machine.

While in the above illustration the percentage of normally beaten kraft has been given as 60%, it is of course understood that this amount may be increased or decreased, and the percentage of gelatinous fibre decreased or increased within fairly wide limits, depending upon the type of paper being prepared. Sheet material and paper made in accordance with the above example may or may not contain sizing materials.

Instead of reducing the Mitscherlich pulp to a jelly-like or gelatinous state by a protracted beating, the same gelatinous condition may be obtained by beating the pulp for a lesser period of time in the presence of an alkaline substance such as caustic soda or sodium silicate. Suitable proportions are approximately 20 lbs. of sodium silicate to 1000 lbs. of cooked pulp, this giving not more than 2% of silicate on the dry pulp. The pulp is then beaten until it has assumed the gelatinous condition. The amount of time required to reach the desired step of hydration will of course be somewhat dependent upon the type of beater and upon the nature of the pulp selected. With a fast type of beater and a Mitscherlich sulphite pulp properly prepared, a satisfactory hydration may be obtained after three hrs. of beating.

This gelatinized fibre may be styled chemically hydrated fibre, in contrast with the mechanically hydrated fibre which is obtained by a prolonged beating in the absence of any chemical reagents. This chemically hydrated gelatinous fibre may be blended with normally beaten pulp after the manner of the first example.

In either case, using the mechanically or chemically gelatinous pulp in admixture with normally beaten pulp, sizing materials, including ordinary rosin size, may be added prior to forming the pulp into sheets. Commercial rosin size may be added to give say 20 lbs. of rosin per 1000 lbs. of pulp, this requiring approximately 40 lbs. of the commercial size. After this has been thoroughly distributed throughout the beaten pulp, 40 lbs. of paper maker's alum are added to the beater, this amount being sufficient to make the furnish slightly acid. The addition of size and alum are in conformance with standard practice.

Where a high degree of flexibility is required, and at the same time high dielectric strength, it is preferred to add a dispersed rubber to the contents of the beater prior to making into sheets. In case the product is to contain sizing, the rubber dispersion is added before the size is introduced. In the preparation of flexible insulating papers containing dispersed rubber, the following procedure may be utilized. The mixture of normally beaten fibre and gelatinized fibre is prepared in the above described manner, and beating is continued until the proper state of hydration or uniformity of mixture has been reached. The beater roll is then raised off the bed plate. A quantity of rubber latex, sufficient to give 50 lbs. of dry rubber per 1000 lbs. of dry pulp is then added, the contents of the beater having been previously made alkaline. If desired a protective colloid, such as glue, casein and acetylated starch viscose, or their equivalents, etc. may be introduced prior to the addition of rubber, simultaneously therewith or after the rubber dispersion has been added. The beater roll in its elevated position is then continued in rotation and made to serve as a mixing device to distribute the rubber latex throughout the beaten pulp. If size is to be incorporated, it may now be added. After the rubber latex, and the size (if size be used) are thoroughly distributed throughout the pulp, a dilute solution of a suitable coagulant such as paper maker's alum is then slowly and carefully added to the contents of the beater, meanwhile continuing the rotation of the beater roll. By the slow addition of the coagulant, the rubber is first agglomerated on the fibres and finally coagulated or anchored thereon. If desired, the coagulant may be added in two stages, in the first of which about two-thirds of the total quantity of alum are added

slowly, followed by a brief interval of mixing, and then the addition of the remainder of the alum. With the above proportion of rubber, 100 lbs. of alum will be satisfactory, this amount being sufficient to make the furnish decidedly acid to an indicator such as litmus. The mixture of normally beaten and gelatinous pulp containing rubber may be made into sheets up to 30-35 points thickness on any of the continuous types of paper machines, and thicker sheets may be made on special types of machinery, such as the wet machine.

The flexible insulating paper thus made contains 60% of normally beaten kraft, 40% of gelatinous fibre, and 5 parts of dry rubber per 100 lbs. of pulp. This product has a piercing potential of approximately 325 volts per mil. With 80% kraft and 20% jelly the piercing potential is 225 volts per mil. By calendering the paper this value may be increased to 270. The paper is highly flexible, and particularly extensible at the edges. This property of marginal extensibility is particularly valuable where the paper is to be wound upon a conductor or upon any other supporting body. By virtue of the marginal extensibility the paper or sheet material in strip form may be lapped to give tight joints, without tearing at the edges, or wrinkling the strip. Another property possessed by this sheet material may be described as surface drag. When the paper or sheet material is wound upon a conductor or supporting material, the adhesiveness or drag on the surface of the material makes it possible to wind very tightly, and tends to hold the windings in place, thus eliminating slippage with the attendant exposure of the conductor. These particular properties, surface drag and marginal flexibility, are not possessed by ordinary insulating papers, for these slip, will not wrap tightly, show a tendency to wrinkle or tear at the edges. In fact the ordinary insulating papers cannot be used unless they are held in place by a protective coating, usually a braided jacket or its equivalent.

The presence of the rubber in the insulating papers and sheets serves to increase the wet tensile to a figure which is approximately equal to the wet tensile strength of ordinary insulating paper of the parchment type.

By varying the amount of rubber employed, the proportion of normally beaten and jelly like pulp, a wide range of mechanical properties, including flexibility, extensibility, tensile strength, tear resistance, folding, etc. may be obtained. As the proportion of kraft or normally beaten fibre is increased, it will be found that the strength of the paper also increases, but the dielectric strength is reduced. Conversely as the proportion of gelatinous fibre is increased the dielectric strength increases, and the tensile

strength decreases somewhat. With greater percentages of rubber the flexibility of the paper is augmented, with but little change in dielectric strength. Wet tensile strength 5 is increased by the inclusion of larger percentages of rubber, and both surface drag and marginal extensibility are increased.

In instances where permanent flexibility is not required, the gelatinous or jelly-like 10 pulp may be used without normally beaten fibre in the production of insulating sheets. In this instance the degree of mechanical or chemical hydration or both may be controlled to give a pulp which is almost entirely gelatinous, or which retains a sufficient percentage 15 of fibre which has undergone only a normal amount of hydration, so that the resultant sheet will have a sufficient amount of strength for the nature of the service required of it. 20 If flexibility is required for winding or otherwise applying, but is not an essential property after the installation, the paper or sheet may be dampened slightly in order to make it sufficiently flexible during the period of 25 installation, it being understood that upon drying the paper is comparatively brittle. This product can be molded if desired, and preferably the molding is done with the jelly-like or gelatinous mass after the greater part 30 of the mechanically included water has been removed and most of the shrinkage has taken place. Molded insulating articles made from this pulp can be machined, turned, sawed, drilled, polished, and engraved with a high 35 degree of facility. The cuttings or waste pieces or even the dried powdered product itself may be used in a dry state with or without a binder such as hard wood pitch for packing, or puttying or otherwise filling irregular spaces which are required to be 40 insulated. By so utilizing the dry material it is frequently possible to effect an economy in the amount of high-grade insulating paper which would otherwise be required to secure 45 proper insulating in locations which are not easily accessible.

The flexibility of the insulating paper described in the immediately preceding paragraph may be increased by the addition of 50 dispersed rubber. The procedure for introducing the rubber may be the same as that described for introducing dispersed rubber into mixtures of normally beaten fibre and jelly-like fibre. When rubber is combined 55 with the gelatinous pulp, an insulating paper may be prepared which has a fair amount of flexibility, sufficient for many purposes, and a high dielectric strength. With 50 lbs. of dry rubber per 1000 lbs. of dry pulp flexible 60 insulating papers have been made to show a dielectric strength of 1150 volts per mil.

While in the above illustrations bleached or unbleached sulphite pulp cooked according to the Mitscherlich process has been described, it is understood that instead of the

slow Mitscherlich cook, a more rapid cook may be employed in the present invention provided it will give a proper degree of hydration without too greatly impairing the strength of the pulp. Kraft pulp may be 70 used, but more time is required to hydrate kraft pulp than the above described sulphite pulp. However, kraft pulp is suitable as the source of the fibre which is to receive only the normal amount of beating. Vegetable 75 fibres including cotton may be utilized to advantage in the above examples, as one means of securing strong sheets.

The invention contemplates the use of rubber in any of its dispersions, natural, synthetic or artificial, or mixtures of any of these. The rubber itself may comprise the globular rubber particles occurring in natural latex, or it may be an artificial latex comprising dispersed crude rubber, vulcanized 80 rubber, reclaimed rubber, separately or in admixture with each other, and may include mixtures of these together with other rubber-like gums, etc. Compounding ingredients 85 may be included in the rubber dispersion, and particularly those ingredients which have the property of imparting or increasing dielectric strength. For example it may be desirable to employ as compounding ingredients 90 certain of the oils, fats, waxes, resins. Vulcanizing materials and accelerators may be added if desired, or the rubber may be in the form of a dispersion of vulcanized rubber, 95 that is a vulcanized latex.

In the claims the term "dispersed rubber" 100 is description of any of the dispersions mentioned in the preceding paragraph. Paper making ingredients, without qualification, comprehends those ingredients which are added to impart special properties to fibrous sheets, as for example waterproofness, flexibility, pliability, denseness, of sheet, etc., and these ingredients include sizing materials in addition as well as special materials which may be added in any suitable form, as solutions or dispersions, or otherwise. Preferably, but not necessarily, such ingredients are added prior to the introduction of the rubber dispersion although they may be combined with the dispersion. 110

Having thus described our invention, what we claim and desire to protect by Letters Patent is:

1. A method of making flexible insulating sheet material which comprises hydrating paper making pulp to a gelatinous condition, combining normally hydrated pulp therewith, mixing dispersed rubber therewith, and forming into sheets. 120

2. A method of making flexible insulating sheet material which comprises combining a slowly cooked gelatinized paper making pulp with paper making pulp which has been hydrated to a considerably less degree, mixing dispersed rubber and paper making in- 125

- gredients therewith, and forming into sheets.
3. A method of making flexible insulating sheets which comprises hydrating paper making pulp to a gelatinous condition, combining normally hydrated pulp therewith, introducing a protective colloid and a rubber dispersion therewith, and forming into sheets.
4. A method of making flexible insulating sheets which comprises hydrating paper making pulp to a gelatinous condition, combining normally hydrated pulp therewith, depositing dispersed rubber thereupon in the presence of a protective colloid and sizing material, and forming into sheets.
- 15 5. A method of making flexible insulating sheets which comprises hydrating paper making pulp to a gelatinous state in the presence of an alkaline material, combining normally beaten pulp therewith, mixing dispersed rubber therewith, and making into sheets.
- 20 6. A method of making flexible insulating sheets which comprises hydrating paper making pulp to a gelatinous state in the presence of an alkaline material, combining normally beaten pulp therewith, adding sizing material and dispersed rubber thereto, and making into sheets.
- 30 7. A method of making flexible insulating sheets which comprises hydrating paper making pulp to a gelatinous state in the presence of an alkaline material, combining normally beaten pulp therewith, introducing a protective colloid and a rubber dispersion therewith, and making into sheets.
- 35 8. A method of making flexible insulating sheets which comprises hydrating paper making pulp to a gelatinous state in the presence of an alkaline material, combining normally beaten pulp therewith, depositing dispersed rubber thereupon in the presence of a protective colloid and sizing material, and making into sheets.
- 40 9. A method of making flexible insulating sheets which comprises converting paper making pulp to a partially gelatinous condition in the presence of an alkaline material, without greatly decreasing the fibrous strength of the pulp, incorporating dispersed rubber therewith, in the presence of paper making ingredients, and forming into sheets.
- 45 10. A method of making flexible insulating sheets which comprises converting paper making pulp to a partially gelatinous condition in the presence of a soluble silicate, without greatly decreasing the fibrous strength of the pulp, incorporating dispersed rubber therewith, in the presence of paper making ingredients, and forming into sheets.
- 50 11. A method of making flexible insulating sheets which comprises converting paper making fibre to a partially gelatinous condition in the presence of a soluble silicate, incorporating dispersed rubber therewith, in the presence of a protective colloid, and forming into sheets.
- 55 12. A method of making flexible insulating sheets which comprises converting paper making fibre to a partially gelatinous condition in the presence of a soluble silicate, incorporating dispersed rubber therewith, in the presence of sizing materials and protective colloid, and forming into sheets.
- 60 13. As a new product a flexible insulating sheet material comprising normally beaten paper making pulp, gelatinized pulp and dispersed rubber, said sheet being characterized by a close formation, high dielectric strength, and tensile strength.
- 65 14. As a new product a flexible insulating sheet material comprising normally beaten paper making pulp, gelatinized pulp, dispersed rubber and sizing material, said sheet being characterized by its marginal extensibility.
- 70 15. An improved insulating material comprising in combination mechanically hydrated paper making fibre, chemically hydrated gelatinized fibre, rubber latex and sizing, said material being dense, non-porous, and characterized by high dielectric strength.
- 75 16. A flexible insulating sheet material comprising in combination chemically hydrated gelatinous paper making pulp and normally beaten pulp, dispersed rubber, a protective colloid, an alkali, and sizing material, said sheet being characterized by close formation, high dielectric strength and tensile strength, great flexibility, particularly at the edges of the sheet, and comparatively high surface drag.
- 80 17. An insulating material comprising rosin sized gelatinized hydrated vegetable fibre, rubber, and a protective colloid including an acetylated starch.
- 85 18. An insulating material comprising rosin sized gelatinized hydrated vegetable fibre, rubber, and a protective colloid including an acetylated starch and a soluble silicate.
- 90 19. An insulating paper comprising rosin sized highly hydrated cotton fibre, rubber, and a protective colloid including an acetylated starch.
- 95 20. An insulating paper comprising rosin sized highly hydrated cotton fibre, rubber, and a protective colloid including an acetylated starch and a soluble silicate.
- 100 21. A method of improving the service qualities of insulating papers of the type containing hydrated vegetable fibres which comprises adding a dispersion of rubber to a hydrated vegetable fibre beaten to a gelatinous condition in the presence of a soluble silicate and an acetylated starch, mixing the rubber with the fibre, incorporating a paper-sizing material therewith and forming into sheets.
- 105 22. A method of improving the service qualities of insulating papers of the type containing hydrated vegetable fibres which comprises adding a dispersion of rubber to

5 a highly hydrated vegetable fibre beaten in the presence of a soluble silicate and an acetylated starch, mixing the rubber with the fibre, incorporating a rosin size therewith and forming into sheets.

10 23. A method of improving the service qualities of insulating papers of the type containing hydrated vegetable fibres which comprises adding a dispersion of rubber to a highly hydrated vegetable fibre beaten in the presence of a soluble silicate and an acetylated starch, mixing the rubber with the fibre, incorporating a rosin size therewith, coagulating the rubber and size upon the beaten fibre, and forming into sheets.

15 24. A method of improving the service qualities of insulating papers of the type containing hydrated vegetable fibres which comprises adding a dispersion of rubber to a highly hydrated vegetable fibre beaten in the presence of a soluble silicate and an acetylated starch, mixing the rubber with the fibre, incorporating a rosin size therewith, coagulating the rubber and size upon the beaten fibre with an alum solution, and forming into sheets.

20 25. A flexible insulating paper comprising an intimate association of highly mechanically and chemically hydrated cellulosic material, paper-sizing, and rubber, said paper being non-hygroscopic, highly resistant to piercing by electric current, and possessing high wet tensile strength and folding number.

25 26. A method of improving the useful quality of insulating material of the type consisting of hydrated paper-making fibres which comprises dispersing rubber throughout a suspension of gelatinized mechanically and chemically hydrated paper-making pulp, depositing the rubber on the pulp and forming into a sheet.

30 27. A method of improving the service qualities of insulating papers of the type containing gelatinized hydrated vegetable fibres which comprises adding a dispersion of rubber to a gelatinized hydrated vegetable fibre beaten throughout in the presence of a protective colloid, mixing the rubber with the fibre and forming into sheets.

35 28. A method of improving the service qualities of insulating papers of the type containing gelatinized hydrated vegetable fibres which comprises adding a dispersion of rubber to a gelatinized hydrated vegetable fibre beaten throughout in the presence of a protective colloid, mixing the rubber with the fibre, incorporating a paper-sizing material therewith and forming into sheets.

40 29. A flexible insulating paper with high tear resistance comprising normally hydrated fibre bonded and filled in by a highly hydrated pulp and the deposit from a water dispersion of rubber.

45 30. A flexible insulating paper with high

tear resistance comprising normally hydrated fibre bonded and filled in by a mechanically and chemically gelatinized pulp, sizing, and the deposit from rubber latex.

31. A method of making insulating material which comprises beating paper pulp and water in the presence of a hydrating agent until it has assumed a gelatinous state, mixing a water dispersion of rubber therewith, uniformly depositing the rubber on the pulp by slow coagulation, and forming an article from the pulp. 70

32. A method of making insulating material which comprises beating paper pulp in the presence of an alkali until it has assumed a gelatinous state, mixing rubber latex therewith, uniformly depositing the rubber on the pulp by slow coagulation, and forming an article from the pulp. 80

33. A method of making insulating material which comprises beating paper pulp and water in the presence of a hydrating agent until the pulp has assumed a gelatinous state, mixing the pulp with a water dispersion of rubber and a normally hydrated pulp, depositing the rubber on the pulp by slow coagulation, and forming an article from the pulp. 85

34. A method of making insulating material which comprises beating paper pulp in the presence of an alkali until it has assumed a gelatinous state, mixing the pulp with rubber latex and a normally hydrated pulp, depositing the rubber on the pulp by slow coagulation, and forming an article from the pulp. 95

Signed at New York, county and State of New York, this 28th day of July, 1927.

REED P. ROSE.

Signed at New York, county and State of New York, this 28th day of July, 1927. 105

HAROLD E. CUDE.

110

115

120

125

130